

## UNITED STATES PATENT OFFICE

2,078,755

COATING FUEL TO PREVENT DUSTING AND  
PRODUCT THEREOF

Per K. Frolich, Elizabeth, N. J., assignor to Standard Oil Development Company, a corporation of Delaware

No Drawing. Application December 12, 1931,  
Serial No. 580,738

12 Claims. (Cl. 44—6)

This invention relates to improvements in methods of treating solid fuels (coal, coke, briquets, and the like) with substances adapted to render the fuels relatively non-dusting. For this and other purposes according to the present invention sulfonic acid compounds derived from petroleum, naphthalene sulfonic acids, and the like, are used, either as such or in the form of their salts. These compounds lay the dust present at the time of treatment and prevent or retard surface disintegration or slacking of the fuels.

The terms "sulphonic compound" and "sulfonate" are used herein and in the claims to signify acidic compounds of the type obtained by reaction of an organic compound with strong or fuming sulphuric acid, and salts thereof, respectively, and does not include the so-called "ligno-sulfonic" compounds derived from wood sulfite liquor, a by-product of paper manufacture.

Sulfonic compounds of the type described possess the following properties which make them desirable for treating fuels:

These compounds form tenacious films over the fuel surface. They do not retard combustion. They add slightly to the fuel value of the material and do not result in objectionable smoke production. They are substantially without odor and under normal conditions of use they do not corrode metals nor cause any injury to those handling the fuel. They can be applied in solution (aqueous or organic solvent) by ordinary spray methods. They are available in many oil refineries as waste materials which can be obtained very cheaply. The aqueous solutions applied can be sufficiently concentrated to prevent danger of freezing and binding of the fuel lumps together, or suitable freezing point depressants may be added, e. g. sodium chloride, molasses, etc. When oil solutions are used, substances tending to lower the pour point may be added, for example the substances described in the United States Patent No. 1,815,022 to G. H. B. Davis, granted July 14, 1931. When dried upon the fuel in presence of air the sulfonic compounds are not readily dissolved by contact with water. The blackness and luster of the fuel is improved by treating with the sulfonic compounds.

Coal, coke, briquets or the like which have been discolored on storage may also be improved in appearance by treatment with the sulfonic acids or sulfonates. The sulfonic compounds when added to the discolored coal or other solid fuel coat the fuel and conceal the discoloration.

Coal which has been previously artificially colored may also be treated with these sulfonic compounds in order to prevent dusting. In this case the amount of treating material used is not sufficient to completely cover all of the coal particles, thus leaving some of the characteristic coloring material to act as a distinguishing feature.

I am aware that various substances having certain of the above-mentioned properties have been used heretofore to make solid fuels non-dusting, for example, mineral oils as such, emulsified mineral oils, magnesium chloride, calcium chloride, etc.

In accordance with the present invention the improved treating agents may be applied by any usual spraying means. This is in general preferred although the fuel may be immersed in the solution or otherwise brought into contact with it. An advantageous way of carrying out the invention is to prepare a 5-15% solution of the sulfonic compound in water (referring first to water soluble compounds) and spray it on the coal or other fuel as it passes through the rotary sizing screens. For example, a solution of 15% of sodium sulfonate derived from petroleum and slightly acid is desirable. Generally, about  $\frac{1}{3}$  to 2 pounds of solid sulfonic compounds in solution are necessary for treating one ton of coal to form a satisfactory superficial layer over the lumps. A somewhat larger quantity is required for treating coke or other absorptive fuel. The treating agent is most conveniently supplied to the trade in concentrated form, say about 45% sulfonic compounds and 55% water. This material especially the neutralized sulfonic acids, may also be dried by a spray drier or the like and the powder dissolved in the necessary amount of water at the place where the fuel is to be treated.

In the foregoing description reference has been made to the water soluble sulfonic compounds which are well known products of the treating of heavy petroleum fractions with fuming or concentrated sulfuric acid for the manufacture of white oils and certain lubricating oils. These sulfonic compounds are separated in the sludge from the acid treatment. The sludge is washed with water with or without the addition of live steam and the acids are used as such or after neutralizing them with a suitable base which may be an alkali or alkaline earth metal (herein referred to generally as alkali), preferably sodium or calcium. It is highly advantageous to remove as much sulfuric acid by such

treatment as possible, not only because of the corrosive action of the latter and the increase in viscosity which it gives the solution, but also because of the white coloration produced by the sodium sulfate when a neutralized sludge is allowed to dry on the fuel. Generally, the sulfuric acid content should be controlled to between 2-15%.

The oil soluble sulfonic compounds are also suitable for making coal non-dusting. These compounds are retained by the oil after the sulfuric acid treatment and are removed from the oil by washing with an organic solvent such as isopropyl alcohol. The alcohol solution containing sulfonic acids may be used either with or without completely or partially neutralizing the sulfonic acids, for treating coal and other fuels. Alternatively, the sulfonic acids or their salts may be separated and supplied either in alcohol or water solution or in alcohol-water solution. An equivalent method is to dissolve the sulfonic compounds in gas oil or other hydrocarbon oil the use of which would not involve an undue fire hazard when spraying solid fuel. When the fire hazard is not a consideration, low boiling oils such as gasoline, naphtha, etc., may be used as solvents for the sulfonic compounds.

The method described above is satisfactory for sulfonic acids obtained by treating lubricating oil (white oil) fractions with sulfuric acid. However, when another fraction of petroleum oil, such as bottoms stock, (cylinder stock, etc.), is treated with sulfuric acid, the following procedure is adopted to make a suitable coal treating material: The sludge is first washed with a small amount of water to remove sulfuric acid. The sulfuric acid (bottom layer) is drawn off, additional water is added to the top layer and the water soluble sulfonic acids are extracted and may be used directly as such or partially neutralized to treat solid fuel.

If necessary, the solvent for the sulfonic compounds may be heated to any temperature short of its atmospheric boiling point, or heated under pressure, to bring the sulfonic compounds readily into solution. In general such heating is not necessary.

The proportions of the oil soluble sulfonic compounds to be used may be the same as described for the water soluble compounds. In both cases it will be understood that considerable variation in the concentration is permissible, a higher concentration being required for fuels having a more pronounced tendency to form dust. The presence of other substances is not precluded in the coating composition so long as the sulfonic compounds exert the essential non-dusting effect.

The sulfonic compounds are capable of carry-

ing dyes of various kinds and fuels may be simultaneously dyed and rendered non-dusting.

Various changes and alternative compositions may be adopted within the scope of the appended claims in which it is my intention to claim all novelty inherent in the invention as broadly as the prior art permits.

I claim:

1. Method of treating solid carbonaceous fuels comprising coating them with a material containing a hydrocarbon sulfonic compound adapted to retard the formation of dust and substantially free of tar. 10

2. Method of treating solid carbonaceous fuels comprising coating them with a separated sulfonic compound derived from acid treated petroleum, adapted to retard the formation of dust, and substantially free of tar. 15

3. Method of treating solid carbonaceous fuels comprising coating them with a material selected from the class consisting of sulfonic acids separated from acid treated petroleum and their neutralized products. 20

4. Method of treating solid carbonaceous fuels comprising coating them with water-soluble sulfonates separated from acid treated petroleum and substantially free of tar. 25

5. Method of treating solid carbonaceous fuels comprising coating them with a water suspension of oil-soluble sulfonates derived from acid treated petroleum. 30

6. Method of treating solid carbonaceous fuels comprising coating them with hydrocarbon sulfonic compounds in the amount of  $\frac{1}{3}$  to 2 lbs. of solid sulfonic compounds per ton of fuel. 35

7. Method of treating solid carbonaceous fuels comprising coating them with a water solution containing 5 to 15% of hydrocarbon sulfonic compounds. 40

8. Method for inhibiting the dusting and surface slacking of coal and coke in lump form, comprising wetting the surface of the lumps with an aqueous solution of a hydrocarbon sulfonate. 45

9. Method according to claim 8 in which said sulfonate is separated from a washed and neutralized petroleum acid sludge.

10. An improved fuel composition comprising a solid fuel, the surface of which is coated with a sulfonic compound derived from petroleum, by sulphuric acid treatment thereof and free from the major amount of tar and sulphuric acid. 50

11. A composition according to claim 10 in which the solid fuel is coated with an aqueous solution of a neutralized sulfonic compound. 55

12. A composition according to claim 10 in which the solid fuel is coated with a neutralized sulfonic compound in an organic solvent.

PER K. FROLICH.